

## 1

2,733,207

## PHOSPHORUS AND SULFUR CONTAINING ANTIOXIDANT

Ferdinand P. Otto, Woodbury, N. J., assignor to Socony Mobil Oil Company, Inc., a corporation of New York

No Drawing. Application January 17, 1952,  
Serial No. 267,009

15 Claims. (Cl. 252—32.7)

This invention relates to reaction products capable of improving the oxidation- and corrosion-resisting properties of mineral lubricating oils. It is more particularly concerned with reaction products of phosphorus sulfide with alkyl disulfides and thiocyanates, and the metal salts thereof.

As is well known to those familiar to the art, it has been proposed to react many materials with phosphorus sulfides, to produce products capable of improving the properties of lubricants. Thus, there have been reacted with phosphorus pentasulfide olefins of several types, petroleum fractions, terpenes, alcohols, mercaptans, etc. In so far as is now known, however, it has never been known that effective antioxidants can be produced by reacting alkyl disulfides or thiocyanates with phosphorus pentasulfide.

It has now been discovered that certain reaction products of this type impart improved properties to lubricants. It has now been discovered that the reaction products of relatively high molecular weight disulfides or thiocyanates with phosphorus pentasulfide, and metal salts of the disulfide reaction product effectively improve the resistance of mineral lubricating oils to oxidation and to corrosion.

Accordingly, it is a broad object of the present invention to provide lubricants having improved resistance to oxidation and to corrosion. A further object is to provide novel addition agents for mineral lubricating oils. Another object is to provide lubricating oils containing novel phosphorus and sulfur-containing additives. A specific object is to provide reaction products of alkyl thiocyanates or disulfides with phosphorus pentasulfide, and salts thereof, and mineral lubricating oils containing them. Other objects and advantages of the present invention will become apparent to those skilled in the art, from the following detailed description.

Broadly stated, the present invention provides a mineral lubricating oil containing a small amount, sufficient to improve the resistance thereof to oxidation, of an antioxidant of the group consisting of (1) a reaction product of an alkyl thiocyanate, having at least about 12 carbon atoms per alkyl radical, with phosphorus pentasulfide, (2) the reaction product of an alkyl disulfide, having at least about 12 carbon atoms per alkyl radical, with phosphorus pentasulfide, and (3) an alkaline-earth metal salt of said alkyl disulfide-phosphorus pentasulfide reaction product.

The alkyl thiocyanates and alkyl disulfides which are reacted with phosphorus pentasulfide to produce the reaction products of this invention have the respective formulae,  $RSCN$  and  $R-S-S-R$ , wherein  $R$  is an alkyl radical. The alkyl radicals in the foregoing formulae should contain at least 12 carbon atoms and up to about 34 carbon atoms. These radicals can be straight-chain or branched-chain alkyl radicals. Especially preferred are the alkyl thiocyanates and disulfides having between about 21 and about 34 carbon atoms per alkyl radical, particularly the wax thiocyanates and disulfides. Non-limiting examples of the thiocyanate and disulfide reactants are dodecyl thiocyanate, isododecyl disulfide, tetra-

## 2

decyl thiocyanate, heptadecyl disulfide, octadecyl disulfide, eicosyl thiocyanate, heneicosyl thiocyanate, docosyl disulfide, 2-methyltricosyl thiocyanate, isohexacosyl disulfide, tetracosyl thiocyanate, paraffin wax disulfide, paraffin wax thiocyanate, ozokerite disulfide, ceresin wax thiocyanate, slack wax disulfide, and scale wax thiocyanate.

The alkyl thiocyanates and disulfides contemplated herein are well known to those familiar to the art. Several methods for their preparation are available. For example, a feasible method is described in a copending Otto application, Serial Number 267,008, filed January 17, 1952. Some of these materials are also available commercially. Any alkyl thiocyanate or alkyl disulfide is utilized for the purposes of the present invention, regardless of its source.

The phosphorus pentasulfide reactant also is well known to the art. This compound,  $P_2S_5$ , is readily available from a number of sources, and it is easily prepared. Either chemically pure or commercial quality phosphorus pentasulfide is utilized herein.

In order to ensure complete reaction between the phosphorus pentasulfide reactant and the alkyl thiocyanate or alkyl disulfide, a weight excess of phosphorus pentasulfide should be used. Due to its insolubility in the final reaction product, unreacted phosphorus pentasulfide is readily removed, as by filtration. In general, the amount of phosphorus pentasulfide used will be between about 0.25 mole and about one mole thereof per mole of thiocyanate or disulfide reactant.

The reaction between the phosphorus pentasulfide and the alkyl thiocyanate or disulfide is effected at a temperature of between about 100° C. and about 200° C. The lower temperatures, around about 100° C., yield a product having a relatively high acidity. On the other hand, temperatures of between about 150° C. and about 200° C. favor the formation of reaction products having a relatively lower acidity. For the purposes of this invention, products produced at any temperature within the range 40 predefined are effective antioxidants.

The reaction contemplated herein is usually complete in between about one hour and about five hours. In practice, a reaction time of between about two and about three hours is sufficient. Generally, the higher molecular weight reactants require more time for complete reaction, in accordance with the present invention. Likewise, of course, the reaction time will vary with the reaction temperature selected.

The use of a solvent in the present reaction is not generally necessary. If desired, a hydrocarbon solvent can be used. A solvent is often indicated, however, especially if the final reaction product tends to be viscous, tacky, or waxy. For practical reasons, it is desirable to prepare the reaction product in a mineral oil solvent, thus producing a concentrate, for ease in handling during blending operations. Between about 25 per cent and about 75 per cent, by weight, of the entire solution of oil and product can be mineral oil. Such a mineral oil solvent can be a lighter oil than the mineral lubricating oil to be improved, or it can be substantially the same, or the same. This is a matter of preference with the user.

Due to the complexity of the final reaction products, since the mechanism involved in the present reaction is not known, no structural formulae can be assigned to the reaction products. Accordingly, it will be appreciated that any definition of the reaction products, other than a definition reciting the method of preparing them, is highly inaccurate.

As mentioned hereinbefore, metal salts of the alkyl disulfide-phosphorus pentasulfide reaction product are also effective antioxidants and anticorrosion agents. The preferred salt-forming metals are the alkaline earth metals,

i. e., barium, calcium, magnesium, strontium, and beryllium. It must be understood, however, that other salt-forming metals, commonly used to prepare mineral oil additives, can be employed and are contemplated herein. Such metals include zinc, aluminum, cobalt, nickel, and the like.

The metal salts of the alkyl disulfide-phosphorus pentasulfide reaction products are substantially neutral salts. In other words, the reaction product is completely neutralized. Salt formation is effected by any of the several methods known to the art. The salts can be formed, for example, by first preparing the alkali-metal, e. g., the sodium salt and then effecting a double decomposition reaction with a soluble inorganic salt of the desired metal, e. g., barium nitrate, calcium chloride, etc. The salts can also be produced by heating the reaction product with an oxide or hydroxide of the desired metal, at temperatures above the boiling point of water, in order to drive off water of neutralization. If desired, a low-boiling solvent, such as, a lower alcohol, benzene, toluene, etc., can be employed, in order to remove water by azeotropic distillation. It must be noted, however, that the particular method selected for salt formation is not a critical factor.

Since the metal salts of the reaction products, as contemplated herein, tend to be viscous or waxy, it is desirable to prepare them in the presence of a mineral oil solvent. Between about 25 per cent and about 75 per cent, by weight, of the final solution of salt and oil, can be mineral oil. As described hereinbefore, the mineral oil solvent can be light or heavy, dependent upon individual preference.

The following specific examples are for the purpose of demonstrating the best methods for preparing the additives of this invention, and to demonstrate the effectiveness thereof. Although wax reaction products are illustrated, it is to be strictly understood that this invention is not to be limited to the specific reactants used in the examples, or to the operations and manipulations involved therein. As those familiar with the art will understand, a wide variety of other reactants and conditions, as defined hereinbefore, can be used.

#### ALKYL THIOCYANATE-P<sub>2</sub>S<sub>5</sub> PRODUCTS

##### Example 1

A mixture of 100 grams of paraffin wax thiocyanate and 15 grams of phosphorus pentasulfide was heated, with agitation, at a temperature of about 100° C., for three hours. The hot reaction mixture was then filtered through filtering clay on a steam-heated funnel, in order to remove unreacted phosphorus pentasulfide. The product thus obtained, i. e., the filtrate, was a brown, waxy material containing, by weight, 14.6 per cent sulfur, 2.4 per cent nitrogen, and 4.04 per cent phosphorus, and having a neutralization number of 93.

The wax thiocyanate employed herein was the product described and defined in Example 2 of the copending application, Serial Number 267,008, filed January 17, 1952.

##### Example 2

A mixture of 63 grams of wax thiocyanate (as defined in Example 1), 7.5 grams of phosphorus pentasulfide, and 63 grams of mineral oil was heated, with agitation, at 170° C. for three hours. The reaction mixture was then cooled to ambient temperature (about 20° C.) and an additional 63 grams of mineral oil was added. The mixture was then filtered through filtering clay on a steam-heated funnel, to remove unreacted phosphorus pentasulfide. The filtered product was a light brown oil containing, by weight, 5.66 per cent sulfur, 1.62 per cent nitrogen, and 1.33 per cent phosphorus, and having a neutralization number of 6.6. The mineral oil used herein was a solvent-refined, Midcontinent stock having a Saybolt Universal Viscosity of 67 seconds at 210° F., a specific gravity of 0.890 and a flash point of 405° F.

#### ALKYL DISULFIDE-P<sub>2</sub>S<sub>5</sub> PRODUCT

##### Example 3

A mixture of 80 grams of wax disulfide and 20 grams of phosphorus pentasulfide was heated, with agitation, at a temperature of about 150° C. for 2.5 hours. The reaction mixture was then filtered to remove unreacted phosphorus pentasulfide. The filtrate was a light brown material, waxy at room temperatures, containing, by weight, 18.8 per cent sulfur and 5.43 per cent phosphorus, and having a neutralization number of 88.5.

The wax disulfide used in this example was the product described and defined in Example 3 of copending application, Serial Number 267,008, filed January 17, 1952.

#### 15 METAL SALT OF ALKYL DISULFIDE-P<sub>2</sub>S<sub>5</sub> PRODUCT

##### Example 4

A mixture of 63 grams of the wax disulfide-P<sub>2</sub>S<sub>5</sub> product of Example 3, 63 grams of mineral oil, 20 grams of barium hydroxide octahydrate, and 100 cubic centimeters of n-butanol was placed in a reaction vessel provided with a mechanical stirrer, thermometer, and a condenser inverted for distillation. The mixture was gradually heated, with agitation, to 150° C., until water and alcohol had ceased to distil (about two hours). The reaction mixture was then cooled to room temperature (about 20° C.) and diluted with about 100 cubic centimeters of benzene. Then the diluted mixture was filtered through filtering clay to remove unreacted barium hydroxide. The solvents (benzene and residual butanol) were removed by topping at 150° C. under reduced pressure. The product was a light brown oil containing, by weight, 5.12 per cent barium, 5.6 per cent sulfur, and 1.48 per cent phosphorus.

#### 35 TEST DATA

##### Example 5

The products described in Examples 1 through 4 were blended, at various concentrations, in portions of a solvent-refined Pennsylvania mineral oil having an A. P. I. gravity of 30.2, a flash point of 435° F., and a viscosity of 63.12 centistokes at 100° F. and of 8.45 centistokes at 210° F. This is a typical motor oil stock. The resultant blends were subjected to the "Bubble Test." In this test, 30 grams of the test oil is placed in a large test tube containing a weighed piece of cadmium-silver bearing, and provided with a gas inlet tube extending to the bottom thereof. The test tube is maintained at 175° C. in a constant temperature bath. Air is blown through the oil, at the rate of two liters per hour, for 22 hours. At the end of the test, the piece of bearing is removed and reweighed. Results are reported in terms of milligrams loss in weight of the bearing. Test results obtained herein are set forth in Table I.

55 TABLE I.—BUBBLE TEST RESULTS

| 60                    | Inhibitor | Percent Conc. | Mg. Loss in Weight |                 |
|-----------------------|-----------|---------------|--------------------|-----------------|
|                       |           |               | Inhibited Oil      | Uninhibited Oil |
| Product of Ex. 1..... |           | 0.125         | 0                  | 23              |
| Do.....               |           | 0.063         | 0                  | 23              |
| Do.....               |           | 0.032         | 2                  | 23              |
| Product of Ex. 2..... |           | 0.5           | 0                  | 23              |
| Do.....               |           | 0.25          | 0                  | 23              |
| Do.....               |           | 0.125         | 0                  | 23              |
| Product of Ex. 3..... |           | 0.25          | 0                  | 21              |
| Do.....               |           | 0.125         | 0                  | 21              |
| Do.....               |           | 0.063         | 0                  | 21              |
| Product of Ex. 4..... |           | 0.25          | 0                  | 28              |
| Do.....               |           | 0.125         | 0                  | 28              |
| Do.....               |           | 0.063         | 0                  | 28              |

##### 70 Example 6

A blend of two per cent, by weight, of the product of Example 4 in a motor oil stock was prepared. This oil is a solvent-refined Pennsylvania stock having an A. P. I. gravity of 31.7, a flash point of 395° F., and

a viscosity of 36.4 centistokes at 100° F. and 5.71 centistokes at 210° F. The blend was subjected to a 36-hour Lauson engine test. The oil was placed in a single cylinder, 4-cycle Lauson engine operated at an oil temperature of 250-260° F., at a speed of 1815 R. P. M., using a 13:1 air-fuel ratio. No oil was added during the test. The neutralization number and the viscosity at 210° F. of the oil are determined at the end of the test. These values, when compared with similar values for the uninhibited base oil, indicate the oxidation tendencies of the test oil under service conditions.

When subjected to this test, the oil blend had a neutralization number of 1.1 and a kinematic viscosity of 6.35 centistokes at 210° F. The uninhibited oil, when subjected to the same test, showed a neutralization number of 7.3 and a viscosity of 8.21 centistokes at 210° F. Accordingly, under the specifications of this test, the test blend is rated as excellent.

#### Example 7

In a solvent-refined Pennsylvania mineral oil base stock having an A. P. I. gravity of about 30.2, a flash point of 435° F., and a viscosity of 63.12 centistokes at 100° F. and 8.45 centistokes at 210° F., was blended two per cent by weight of the product of Example 4. This blend was subjected to the C. F. R. corrosion test. In this test, a C. F. R. fuel test engine, from which all equipment applying only to fuel test work has been removed, is used. Oil at a controlled temperature is delivered by a metering pump from an external heating sump to the test connecting rod bearing, through the drilled crankshaft. All other engine parts are lubricated with oil drawn from the same external sump by a double capacity C. F. R. oil pump. A copper-lead alloy test bearing is placed in the large end of the connecting rod. The jacket temperature is maintained at about 212° F., and the oil temperature at about 285° F. During the test, the compression ratio and engine speed are maintained at 5.5 and 1200 R. P. M., respectively. The engine is operated for a standard time which has been taken as the time (in hours) required for a loss of about 0.200 gram of the copper-lead alloy test bearing when a blank oil is used. The effectiveness of an oil addition agent is measured by the time required for a similar loss when a blend of the same oil and an addition agent is used. The neutralization numbers of the blank oil and of the oil blend were determined after several time intervals, as were the bearing losses of the test bearings. Test results for the blend and for the uninhibited base oil are set forth in Table II.

rust agents, defoamants, and other additives well known to those skilled in the art.

Although the present invention has been described in conjunction with preferred embodiments, modifications and variations are contemplated, as those skilled in the art will readily understand. Such variations and modifications are considered to be within the purview and scope of the appended claims.

#### What is claimed is:

10. 1. As a new composition of matter, an antioxidant selected from the group consisting of (1) the reaction product of an alkyl thiocyanate, having between about 21 and about 34 carbon atoms per alkyl radical, with phosphorus pentasulfide, (2) the reaction product of an alkyl disulfide, having between about 21 and about 34 carbon atoms per alkyl radical, with phosphorus pentasulfide, and (3) an alkaline-earth metal salt of said alkyl disulfide-phosphorus pentasulfide reaction product.
20. 2. The reaction product of an alkyl thiocyanate, having between about 21 and about 34 carbon atoms per alkyl radical, with phosphorus pentasulfide.
30. 3. The reaction product of a paraffin wax thiocyanate with phosphorus pentasulfide.
40. 4. The reaction product of an alkyl disulfide, having between about 21 and about 34 carbon atoms per alkyl radical, with phosphorus pentasulfide.
50. 5. The reaction product of a paraffin wax disulfide with phosphorus pentasulfide.
60. 6. An alkaline-earth metal salt of the reaction product of a paraffin wax disulfide with phosphorus pentasulfide.
70. 7. The barium salt of the reaction product of a petroleum wax disulfide with phosphorus pentasulfide.
80. 8. A mineral lubricating oil containing a small amount, sufficient to improve the resistance thereof to oxidation, of an antioxidant selected from the group consisting of (1) the reaction product of an alkyl thiocyanate, having between about 21 and about 34 carbon atoms per alkyl radical, with phosphorus pentasulfide, (2) the reaction product of an alkyl disulfide, having between about 21 and about 34 carbon atoms per alkyl radical, with phosphorus pentasulfide, and (3) an alkaline-earth metal salt of said alkyl disulfide-phosphorus pentasulfide reaction product.
90. 9. A mineral lubricating oil containing between about 0.05 per cent and about 10 per cent by weight of an antioxidant selected from the group consisting of (1) the reaction product of an alkyl thiocyanate, having between about 21 and about 34 carbon atoms per alkyl radical, with phosphorus pentasulfide, (2) the reaction product of an alkyl disulfide, having between about 21 and about 34 carbon atoms per alkyl radical, with phosphorus pentasulfide, (3) an alkaline-earth metal salt of said alkyl disulfide-phosphorus pentasulfide reaction product.

TABLE II.—C. F. R. CORROSION TEST

|                         | 20 Hrs.    |        | 41 Hrs.    |        | 47 Hrs.    |        | 63 Hrs.    |        | 85 Hrs.    |        | 107 Hrs.   |        |
|-------------------------|------------|--------|------------|--------|------------|--------|------------|--------|------------|--------|------------|--------|
|                         | G.<br>Loss | N. N.* | G.<br>Loss | N. N.* | G.<br>Loss | N. N.* | G.<br>Loss | N. N.* | G.<br>Loss | N. N.* | G.<br>Loss | N. N.* |
| Uninhibited Oil         | 0.014      | 1.4    | 0.135      | 3.5    | 0.235      | -----  | 0.025      | 2.8    | 0.073      | 3.6    | 0.181      | 4.0    |
| Oil+2% Product of Ex. 4 | 0.005      | 0.9    | 0.009      | 1.7    | -----      | -----  | -----      | -----  | -----      | -----  | -----      | -----  |

\*Neutralization number.

From the foregoing examples, it will be apparent that the additives of the present invention have excellent anti-corrosion and antioxidant properties. These additives are ordinarily added to mineral lubricating oils at concentrations of between about 0.05 per cent, by weight, and about 10 per cent, by weight. It is preferred to use weight concentrations of between about 0.5 per cent and about 4 per cent.

It will be appreciated that other addition agents can be added to the mineral oil along with the additives of this invention, in order to improve other properties of the oil. Thus, for example, the oil blend can also contain oiliness agents, E. P. additives, V. I. improvers, anti-

65. 34 carbon atoms per alkyl radical, with phosphorus pentasulfide, and (3) an alkaline-earth metal salt of said alkyl disulfide-phosphorus pentasulfide reaction product.

70. 10. A mineral lubricating oil containing a small amount, sufficient to improve the resistance thereof to oxidation, of the reaction product of an alkyl thiocyanate, having between about 21 and about 34 carbon atoms per alkyl radical, with phosphorus pentasulfide.

75. 11. A mineral lubricating oil containing a small amount, sufficient to improve the resistance thereof to oxidation, of the reaction product of a paraffin wax thiocyanate with phosphorus pentasulfide.

12. A mineral lubricating oil containing a small

amount, sufficient to improve the resistance thereof to oxidation, of the reaction product of an alkyl disulfide, having between about 21 and about 34 carbon atoms per alkyl radical, with phosphorus pentasulfide.

13. A mineral lubricating oil containing a small amount, sufficient to improve the resistance thereof to oxidation, of the reaction product of a paraffin wax disulfide with phosphorus pentasulfide.

14. A mineral lubricating oil containing a small amount, sufficient to improve the resistance thereof to oxidation, of an alkaline-earth metal salt of the reaction product of a paraffin wax disulfide with phosphorus pentasulfide.

5  
10

15. A mineral lubricating oil containing a small amount, sufficient to improve the resistance thereof to oxidation, of the barium salt of the reaction product of a petroleum wax disulfide with phosphorus pentasulfide.

References Cited in the file of this patent

UNITED STATES PATENTS

|           |              |       |               |
|-----------|--------------|-------|---------------|
| 2,150,400 | Rosen        | ----- | Mar. 14, 1939 |
| 2,169,700 | Loane et al. | ----- | Aug. 15, 1939 |
| 2,209,440 | Adams et al. | ----- | July 30, 1940 |
| 2,316,091 | White        | ----- | Apr. 6, 1943  |
| 2,516,119 | Hersh        | ----- | July 25, 1950 |